

## UNITED STATES PATENT OFFICE

2,230,556

## FOAM SUPPRESSOR FOR SOLUBLE OILS

John C. Zimmer, Hillside, and George M. McNulty, Union, N. J., assignors to Standard Oil Development Company, a corporation of Delaware

No Drawing. Application January 11, 1938,  
Serial No. 184,382

6 Claims. (Cl. 252—42)

This invention relates to mineral oil emulsions, especially those used for metal working, and is more particularly concerned with agents to prevent or retard the foaming thereof.

5 Mineral oil emulsions are used in metal working such as the cutting and grinding of gears, tools, crank-shafts, ball bearings, pistons, etc. These emulsions ordinarily consist of a mineral oil, an emulsifying agent and water.

10 The mineral oil may be a light lubricating fraction of petroleum, a spindle oil, white oil or similar type of oil. Distillate oils derived from paraffinic or naphthenic crudes and having Saybolt viscosities at 100° F. between 60 and 200

15 seconds are generally suitable. The emulsifying agent may be a sodium, potassium or "onium" base naphthenate or sulfonate. Organic naphthenate soaps such as di- and triethanolamine naphthenate may also be used. It is generally preferable to use a mixture of naphthenates and sulfonates, say in a ratio of 1 part naphthenate to 4 parts sulfonates. The naphthenates are found to cause excessive foaming and are also more water soluble than the sulfonates. From

20 5 to 40% by weight of the emulsifying agent based on the mineral oil may be used.

It is found that these mineral oil emulsions when agitated and stirred up as they must be in metal working generate considerable foam

30 which is not only troublesome to work with but also causes overflow of the reservoirs and tanks from which the emulsion is supplied.

Several methods for preventing foaming of mineral oil emulsions have been proposed here-  
35 tofore. The usual method is to prepare a com-  
paratively unstable product, thus producing emul-  
sions which separate free oil. This free oil acts  
to some extent as a foam suppressor. The prin-  
cipal disadvantage of this method, however, is  
40 that unstable emulsions tend to separate com-  
pletely under prolonged service.

Another method is to add aluminum stearate or stearic acid to the soluble oil. These mate-  
rials are not especially satisfactory because the  
45 soda present either as free alkali or formed  
by hydrolysis of sodium sulfonate or naphthenate  
soaps tends to displace the aluminum or react  
with the stearic acid to form sodium stearate.  
This sodium stearate tends to cause gelling or  
50 solidification of the soluble oil which, of course,  
is highly objectionable.

The present invention is directed to a new  
method for suppressing the foaming tendency of  
soluble oils. The nature of this method will  
55 fully be understood from the following description:

We have found that waxes of acids having  
more than 22 carbon atoms and containing from  
5 to 50% of free acid having at least 22 carbon  
atoms have the property of suppressing or sub-  
60 stantially preventing the foaming of soluble oil

emulsions. The most suitable wax of this type  
is montan wax, but other waxy derivatives of  
montan wax such as waxes known as "OP" and  
"Z" waxes manufactured and sold by the I. G.  
Farbenindustrie A. G. of Germany are also suit-  
able. These waxes are added to the soluble oil  
in amounts between .001% and about 0.5% by  
weight. The amount of wax added in any par-  
ticular case should not, of course, be sufficient to  
cause separation of the wax from the oil at nor-  
mal temperatures. It is preferable to heat the  
soluble oil to about the melting point of the  
wax and then stir it in vigorously. Overheating  
of the oil should be avoided.

10 These waxes are especially effective in sup-  
pressing foam formation in cases where the emul-  
sifying agent is a naphthenate soap.

15 It will be understood that other materials may  
also be added to the soluble oils besides these  
foam suppressors. For example, dyes, anti-oxi-  
dants, polymer thickeners, resins or, in fact, any  
20 of the usual addition agents for hydrocarbon oils  
may be added without interfering with the ac-  
tion of the waxes.

25 To illustrate the method, a soluble oil con-  
taining a mixture of sulfonate and naphthenate  
soaps as an emulsifying agent is mixed with 40  
parts of water to form an emulsion. To another  
portion of soluble oil about 0.01% montan wax  
30 is added and emulsified with 40 parts water.  
The two emulsions are tested for foaming using  
a Mixmaster agitator.

The following results are obtained:

## Mixmaster foaming test

700 R. P. M. for 10 minutes. 500 cc. sample.

|                              | Foam in-<br>crease in<br>volume | Time for foam<br>to break | Percent |
|------------------------------|---------------------------------|---------------------------|---------|
| 1 Emulsion                   |                                 | 20 minutes.               | 160     |
| 2 Emulsion +0.01% montan wax |                                 | 1-2 seconds               | 0       |

45 In another experiment various quantities of  
wax identified as "OP" wax manufactured by  
the I. G. Farbenindustrie A. G. were added to  
the soluble oil containing naphthenate soap.  
These samples were tested in the Mixmaster as  
above and the following results obtained:

|                           | Foam in-<br>crease in<br>volume | Time for<br>foam to<br>break | Percent | Minutes |
|---------------------------|---------------------------------|------------------------------|---------|---------|
| Emulsion                  |                                 |                              | 160     | 20      |
| Emulsion +0.005% "OP" wax |                                 |                              | 70      | 25      |
| Emulsion +0.010% "OP" wax |                                 |                              | 40      | 22      |
| Emulsion +0.02% "OP" wax  |                                 |                              | 30      | 7       |

These results show that as little as 0.01% of montan wax and as little as 0.02% of "OP" wax will markedly reduce the foaming tendency of the soluble oil when emulsified.

5. Following are formulae for typical soluble oils prepared in accordance with the present invention:

## No. 1

|                     | Per cent |
|---------------------|----------|
| 10 Sodium sulfonate | 12.00    |
| Naphthenic acids    | 3.00     |
| Sodium hydroxide    | 0.50     |
| Alcohol             | 0.50     |
| Water               | 2.00     |
| 15 Montan wax       | 0.05     |
| Paraffin oil        | 81.95    |

## No. 2

|                     | Per cent |
|---------------------|----------|
| 20 Sodium sulfonate | 12.00    |
| Rosin               | 4.60     |
| Sodium hydroxide    | 0.50     |
| Alcohol             | 0.50     |
| Water               | 2.00     |
| 25 Montan wax       | 0.05     |
| Paraffin oil        | 80.35    |

This invention is not limited by any theories of the mechanism of the foaming nor by any details which have been given merely for purposes 30 of illustration, but is limited only in and by the following claims in which it is intended to claim all novelty inherent in the invention.

We claim:

1. Composition of matter comprising a mineral soluble oil containing a small per cent of an emulsifying agent selected from the class consisting of alkali naphthenates, alkali sulfonates, and mixtures of alkali naphthenates and alkali sulfonates and having the property 35 of producing a substantial amount of foam under service conditions and a small percent of a

mineral ester wax of an acid having at least 22 carbon atoms in amount sufficient to reduce the foaming tendency of said oil.

2. Composition of matter comprising a mineral oil, a small percent of an emulsifying agent 5 selected from the class consisting of alkali naphthenates, alkali sulfonates and mixtures of alkali naphthenates and alkali sulfonates, said emulsifying agent being present in sufficient amount to produce a stable emulsion but also to 10 cause substantial amounts of foam, and a small percent of an ester wax of an acid having at least 22 carbon atoms containing at least 5% of free acid having at least 22 carbon atoms in amount sufficient substantially to reduce foam 15 formation.

3. Composition of matter comprising a mineral oil, a small percent of an emulsifying agent selected from the class consisting of alkali naphthenates, alkali sulfonates and mixtures of alkali 20 naphthenates and alkali sulfonates, and a small percent of montan wax in amount sufficient substantially to reduce foam formation.

4. Composition of matter comprising a mineral oil, a small percent of an alkali naphthenate 25 and between 0.001 and 0.5% by weight of montan wax.

5. A non-foaming emulsion comprising water, a mineral oil, a small percent of an alkali naphthenate, and between 0.001 and 0.5% of montan 30 wax.

6. A non-foaming emulsion comprising water, a mineral oil, from 5 to 40% by weight of an emulsifying agent selected from the class consisting of alkali naphthenates, alkali sulfonates, 35 and mixtures of alkali naphthenates and alkali sulfonates, and between 0.001 and 0.05% montan wax.

JOHN C. ZIMMER.  
GEORGE M. McNULTY.